

July 31, 1951

M. J. MacDONALD ET AL

2,562,726

CREMATORIAL URN

Filed Aug. 25, 1943

2 Sheets-Sheet 1

FIG. 1.



FIG. 2.



FIG. 4.



FIG. 3.



FIG. 5.



INVENTORS  
MURRAY J. MacDONALD  
CARL SCHWENDLER  
CHRISTOPHER S. SCHWENDLER  
BY

*W. Theodore Simmons*  
ATTORNEY

43-64

July 31, 1951

M. J. MacDONALD ET AL  
CREMATORY URN

2,562,726

Filed Aug. 25, 1943

2 Sheets-Sheet 2

FIG. 6.



FIG. 7.



FIG. 8.



INVENTORS  
MURRAY J. Mac DONALD  
CARL SCHWENDLER  
CHRISTOPHER S. SCHWENDLER  
BY

*M. Theodore Scammons*  
ATTORNEY  
43-62

## UNITED STATES PATENT OFFICE

2,562,726

## CREMATORI URN

Murray J. MacDonald, Chappaqua, Carl Schwendler, Woodside, and Christopher S. Schwendler, Elmhurst, N. Y., assignors to National Casket Company Incorporated, Long Island City, N. Y.

Application August 25, 1943, Serial No. 500,179

6 Claims. (Cl. 27—1)

1

Our invention relates to containers, and more particularly to that type of container known as a crematory urn. Such urns normally are used to hold the ashes of a cremated body, and are retained in mausoleums, or elsewhere, and occasionally are interred in the ground.

Heretofore crematory urns have been made of various metals, which have been expensive to manufacture, or of tiles cemented together which, while less expensive to manufacture, lack the stability of structure and appearance demanded commercially, and are subject to other objections, such as the difficulty of hermetically sealing the same. Furthermore, no chemically inert liner has been provided to date, and insofar as we are aware, these urns have not been made of hardenable plastic compositions.

It is one object of our invention to provide a crematory urn made of a hardenable plastic composition; and which has a hard, smooth, finely textured outer surface that may be finished in any suitable manner, such as is done when painting or lacquering a wooden or metal article. Thus, bronze, silver and other finishes may be successfully simulated, such as an ivory finish.

It is another object of our invention to provide an improved construction of crematory urn.

It is still another object of our invention to provide a crematory urn with a suitable chemically inert liner for the chamber thereof.

It is a further object of our invention to provide a crematory urn of the above indicated character which is a monolithic structure, having suitable ornamentation cast thereon, and which is nevertheless light in weight, free from warping and cracking, resistant to shocks, stresses and strains, and which is readily hermetically sealed.

It is a further object of our invention to provide an improved construction of crematory urn wherein the hermetically sealed closure is concealed behind a removable portion of the ornamental construction.

Other and further objects of our invention will be understood from the specification taken in conjunction with the accompanying drawings, wherein—

Figure 1 is a perspective view of one form of crematory urn constructed in accordance with this invention.

Fig. 2 is a vertical section taken on the line 2—2 of Fig. 1.

Fig. 3 is a detail in perspective of the closure cap.

Fig. 4 is a vertical sectional view of the as-

2

sembled mold for the construction of crematory urn shown in Figs. 1 and 2.

Fig. 5 is a detail in perspective of the liner support and mold for producing the cap cavity.

Fig. 6 is a vertical sectional view of a modified construction of crematory urn according to this invention.

Fig. 7 is a vertical sectional view of a still further modified form of crematory urn according to this invention, and

Fig. 8 is an end elevation of the crematory urn of Figs. 6 and 7.

While there is shown and described in this specification the best forms and methods now known to us for carrying out our invention, it will be apparent that various modifications may be made in the plastic composition and its proportions, as well as in the construction and arrangement of parts, within the spirit and scope 20 of the invention as described in this specification and as set forth in the appended claims.

Referring to Figs. 1 to 5, the crematory urn 11 there shown comprises side walls 12, top 13 and an enlarged base 14.

This urn is formed of a hardenable plastic composition to be more fully described hereinafter, and it will be noted that the top 13 has a suitable ornamental shape, and that the side walls 12 are provided with appropriate ornamentation, indicated at 15, leaving large blank areas on the sides for suitable inscription, or the like. The ornamental shape and the surface ornamentations are cast integral with the body by means of a suitably shaped mold, and it will be understood that other shapes and other ornamentations may be used as desired by the manufacturer.

The crematory urn 11 is hollow, as seen in Fig. 2, and is provided with a glass liner 16. The bottom of the urn 11 is provided centrally with an apertured recess 17 into which space the threaded end 18 of the liner 16 projects. The open end of the liner 16 is closed by a cap 19, which also may be formed of the hardenable plastic composition referred to, which fills the recess 17 and has a screw threaded hollow, as indicated at 21, to receive the projecting screw threaded end of the liner 16. A glass, rubber or felt disc 20 may be inserted in the bottom of the hollow to cover the open end of the liner 16. The cap 19 also is provided with a pair of finger holds 22 by means of which the cap may be screwed in place; and when the urn ashes have been deposited in the urn, the cap is suitably sealed in place by a plastic cement, to be described, and indicated at 23, the cement preferably being of a nature to unite the

cap 19 and the urn 11 in a monolithic structure.

For a suitable hardenable plastic composition, meeting all of the requirements of the particular service as well as the requisite economy of manufacture, we prefer a plastic which provides a hard, smooth, finely textured outer surface, and one which can be directly painted, lacquered, or similarly decorated, as is usually done for articles made of wood or metal, so that the article will be commercially acceptable without any special and expensive treatments of the outer surface. The plastic must be sufficiently dense and have an internal structure that will adequately distribute shocks, strains and stresses evenly over a wide area, to prevent excess loading at any one point, and at the same time the plastic in its hardened state must not be brittle, should not be subject to cracking or warping, and desirably should be chemically inert to moisture and acids, especially those encountered in the air and ground.

The plastic composition which we have found suitable is an oxychloride cement containing various fillers enhancing the desirable characteristics.

In our present form, the surface of the urn is formed of an oxychloride cement having certain fillers which enable the urn to have the hard, smooth, finely textured outer surface we prefer, and this surface may be backed by a complementary oxychloride cement having predominately cellular fillers whereby the mass and article have a lighter weight, but at the same time the two materials unite into a monolithic structure, or it is entirely practical and feasible to make the urn entirely of the aforesaid surface composition.

One formula for the surface composition may consist of the following ingredients, stated in parts by weight: calcined magnesite 40, Silex 50, asbestos (desirably short fibre) 6, diatomaceous earth 4, plasticising fluid 100. The magnesite should all pass through a screen of 325 mesh and the Silex is desirably about the same particle size.

The plasticising fluid may be made according to the formula, stated in parts by weight, magnesium chloride 37.4, magnesium sulphate 8.2, water 54.4.

If desired, a small percentage of a coloring matter, such as iron oxide or carbon black, may be added to this formula, in which case the amount of Silex used is generally reduced slightly, but not over an amount corresponding to that of the added coloring matter.

All of the ingredients of the foregoing composition are mineral in character. It has been found possible to obtain a hardenable plastic composition having the characteristics of the hard, smooth, finely textured outer surface, freedom from warping, inherent strength, resistance to weather and acid conditions, etc., while substituting or adding an organic material, such as wood flour, in the formula. This results in a finished product that is lighter in weight, perhaps more resilient to shocks and stresses, and slightly cheaper to manufacture.

A suitable composition in which wood flour is substituted for the mineral fillers may be made in the following proportions, stated in parts by weight:

Calcined magnesite..... 53.5  
Silex..... 42.7  
Wood flour..... 3.8  
Plasticising solution..... 88.6

The wood flour is very finely ground to approximately 400 screen mesh, or finer.

A suitable backing for the surface material and comprising the bulk of the article may be made according to the following formula, proportions being stated in parts by weight:

|                             |      |
|-----------------------------|------|
| Calcined magnesite.....     | 40   |
| Silex.....                  | 27   |
| Asbestos (short fibre)..... | 12   |
| Diatomaceous earth.....     | 16   |
| Pumice.....                 | 5    |
| Plasticising solution.....  | 81.8 |

In the foregoing backing composition, the magnesite is ground to a fine particle size such as all through a 325 mesh screen, and the other ingredients, when used, are of various sizes, i. e., substantially all the pumice will pass through a 16 mesh screen, the Silex is about the same particle size as magnesite, and the short fibre asbestos has a maximum length of about  $\frac{1}{8}$ '. Other fibres may be substituted for the asbestos, such as hemp fibre, due allowance being made for the difference in porosity and absorptiveness thereof.

Calcium is present in the magnesite as an impurity, and the amount sometimes varies in the commercial product. The magnesium sulphate of the plasticising fluid is varied in an amount to react with the calcium present in the mixture as an impurity so as to convert all this calcium into the inert, insoluble, crystalline calcium sulphate. The dry ingredients are very thoroughly mixed prior to the addition of the plasticising fluid, and are again very thoroughly mixed after the addition of the fluid. Consequently, the calcium sulphate is precipitated in innumerable places throughout the mass; and the viscosity of the mass in all cases is maintained such that the precipitated calcium sulphate does not settle out of the mass but remains at its many points of formation in the hardened composition. It is, therefore, uniformly distributed throughout the resulting product, and one important effect of this is that the calcium sulphate forms a lattice work of crystals throughout the mass of the finished article. This internal structure is useful in distributing over wide areas all shocks, stresses and strains on the material of the finished product. Furthermore, it is believed that this crystalline calcium sulphate formation aids in preventing cracking and warping both during the setting period and after the article is finished.

It will be apparent, therefore, that more or less magnesium sulphate may be needed in the plasticising solution to neutralize the lime impurity, and the amount of plasticiser used may vary from the proportions indicated herein, but the proportions stated have been found to be generally satisfactory.

As in the case of the surface material, the major characteristics of the backing composition may be retained without using all mineral ingredients, as indicated in the above formula. Certain organic fillers have been substituted for the mineral fillers, and examples of such composition which has been found to be satisfactory is as follows, stated in parts by weight:

|                            |      |
|----------------------------|------|
| Calcined magnesite.....    | 40   |
| Silex.....                 | 39   |
| Sawdust.....               | 16   |
| Wood flour.....            | 5    |
| Plasticising solution..... | 78.5 |

In this case also, the magnesium sulphate reacts with the calcium present in the mixture to

convert the same to the crystalline calcium sulphate as described above, and the viscosity of the mix is similar, all with the same effects upon the resultant compositions and products.

With the addition of coloring matter as desired, these so-called backing materials may be used for producing the entire article with, however, a different surface appearance from that of our present preferred form.

In the use of the aforementioned hardenable plastic compositions, the urn is cast without the use of heat and pressure, one method of doing so being illustrated in Fig. 4. A mold consisting of two parts 31 and 32, are suitably bolted or locked together to form a mold cavity. The surfaces of the cavity have the necessary provision for the desired surface ornamentalations such as indicated in Fig. 1. Before the mold halves are clamped together, the surface of each half is coated, as by brushing or otherwise, with a thin layer of one of the surface compositions described above. The mold sections are then clamped together and the lower part 33 of the mold cavity is filled with the plastic material made according to one of the above formulae.

The glass liner 16 is screwed into a block insert 34, which is of a size and shape to provide the recess 17 for the cap 19 as indicated in Fig. 2. The block 34 may have imbedded therein a cap 35 having a screw thread to receive the screw threaded end 21 of the liner 16, but these threads may be molded in the block 34. The block is secured to a cross bar 36 arranged to span the mold cavity and to be secured to the opposite halves thereof, as by stud bolts 36. The assembled glass liner 16 and block 34 are pressed home in the partially filled mold cavity until the cross bar 36 is in position at which time the closed end of the liner is embedded in the plastic composition in the lower part of the mold cavity. When the bar 36 is bolted in place, the liner 16 is properly centered and located in the mold cavity, and the remainder of the mold cavity is then filled up to the level of the bar 36 with the plastic composition. As indicated above, the surface and backing plastic compositions unite into a monolithic structure in the finished article.

The mold is then set aside until the plastic composition takes its final set, which occurs in from 3 to 8 hours, and in which time the glass liner 16 is firmly embedded and mounted in the urn casting. After the final set, the screws 36 are removed, by unscrewing the same from the liner 16, which will leave the cavity 17 in the urn casting with the screw threaded end 21 of the liner 16 projecting into that cavity as indicated in Fig. 2. The mold halves are then unclamped, and the urn casting is set aside to age in open racks in the air, which aging requires from 5 to 20 days.

However, the casting has come out of the mold with the hard, smooth, finely textured, and ornamented outer surface desired in the finished article, and any fine which occurs between the mold halves is easily scraped off before the casting is set away to age. The hard, smooth, finely textured outer surface is indicated at 37 in Fig. 2, and the lighter weight cellular or coarser backing material is indicated at 38, but as explained above, actually there is no delineation between these materials, the showing in Fig. 2 being merely to facilitate the illustration.

With the above explanation, it is not believed necessary to describe the molding of the cap 19. Suffice it to say that it, too, is molded of one of

the hardenable plastic compositions referred to, with proper inserts for forming the screw threads therein to engage the screw threaded end 21 of the liner 16, as shown in Fig. 2, and also to provide for the finger recesses 22. When the urn casting and the cap casting 19 have aged as described above, one of the caps is screwed onto the urn, and the same is ready for finishing.

In all instances, the surfaces of the above described urns are such that they may be finished in the normal manner for the painting or lacquering of wood or metal articles, and a firm bond is had between the composition and the paint or lacquer. Briefly described, after the aging period, sealer and priming coatings may be applied to the urn, and after sanding, the desired color, shading or tinting, and lacquer coatings may be applied, followed by the waxing and rubbing down operations. By such treatment, commercially acceptable crematory urns are obtained in a variety of effects.

When the urn is to be put into use, the cap 19 is removed, the ashes inserted, and then the cavity 17 may have a thin coating of a cement, about to be described, applied thereto before the cap 19 is screwed into place, and thus the urn is hermetically sealed.

This sealing cement may be made according to the following formula, stated in parts by weight:

|    |                    |      |
|----|--------------------|------|
| 30 | Calcined magnesite | 45.8 |
|    | Silex              | 50.7 |
|    | Zonolite           | 3.5  |
|    | Plasticising fluid | 82   |

35 Wood flour can be successfully substituted in the above formula for the Zonolite. We have found that when this cementing composition is used with castings made according to the above formula, the separate interfaces of the assembled cap and urn have lost their identity so that the entire article has become a single hermetically sealed, monolithic structure, similar to a case where the object is cast or molded in one piece originally. Any other cement may be used, such as rubber or casein types.

40 Referring to Fig. 6, the urn 41 again has the hard, smooth, finely textured outer surface 42 and the coarser, predominantly cellular, backing 43. In this case, the glass liner 44 is arranged in the urn so that its open screw threaded end 45 is at one side of the urn casting. This screw threaded end is located in a recess 47 and is closed by a cap 46, similar in construction to the cap 19, except for the addition of an outer cover portion 48. The cover portion is large enough to close the recess 47 and is constructed so as to have a conformation which blends with the ornamental design appearance of the urn.

45 Fig. 7 illustrates an urn which for purposes of this example has the same contour as the urn of Fig. 6. However, in this case, the urn is made of two parts, the top 51 and base 52, these two parts being separately cast in open molds in a manner as described above in connection with Fig. 4, which are subsequently cemented together as by use of the cementing composition described above.

50 The base has a raised central portion 53 having a screw threaded opening 54 therein which receives the closure cap 55, similarly to the other closure caps described. In this case there is no glass liner as indicated at 16 and 44 in the other figures of the drawing, such a liner being unnecessary inasmuch as the plastic compositions described above are inert to moisture and acids,

especially such as will be encountered in the open air and ground.

In this case, when the urn is to be used, the cap 55 is removed, the ashes are inserted through the opening 54, a suitable cementing composition is inserted as indicated at 56, and the cap 55 is screwed home, all as described in more detail in connection with the other figures of this drawing.

In all instances, the hermetic sealing of the 10 cap may be dispensed with.

We claim:

1. In a crematory urn, a hollow body formed of a hardenable plastic composition having a hard, smooth, finely textured outer surface, an 15 opening at one end of said body, a recess surrounding said opening, a liner for said body and embedded in said composition, the liner having a screw threaded end portion projecting through the opening and into said recess, and a closure 20 cap fitting in said recess and having a screw threaded portion engaging the projecting end of the liner to close the same.

2. In a crematory urn, a hollow body formed of a hardenable plastic composition having a hard, smooth, finely textured outer surface, an opening at one end of said body, a recess surrounding said opening, a glass liner for said body, the liner having a screw threaded end portion projecting through the opening and into said recess, and a closure 25 cap fitting in said recess and having a screw threaded portion engaging the projecting end of the liner.

3. In a crematory urn, a hollow body formed of a hardenable plastic composition having a hard, smooth, finely textured outer surface, an opening at one end of said body, a recess surrounding said opening, a glass liner for said body, and a closure 30 cap for said opening fitting in said recess and having a peripheral flange provided with a surface complementary to the surface of the body portion around said recess.

4. In a crematory urn, a hollow body formed of a hardenable plastic composition having a hard, smooth, finely textured outer surface, an opening 45 at one end of said body, a recess surrounding said opening, a glass liner for said body, the liner having a screw threaded end portion projecting through the opening and into said recess, and a closure cap fitting in said recess and having a 50

screw threaded portion engaging the projecting end of the liner, the cap including a cover for said recess and also formed of the hardenable plastic composition and of appearance to blend with the design appearance of the urn body.

5. A crematory urn comprising a hollow glass liner, a body formed of a layer of a coarse hardenable plastic composition in which said liner is embedded and a layer of a hardenable plastic of different composition to provide a hard, finely textured outer surface, the two compositions bonding together into a unitary structure, the glass liner and body being open at one end of the urn, and a closure cap for said opening.

6. In a crematory urn, a hollow body formed of a hardenable plastic composition, the urn having an ornamental outer surface, an opening on one end of said body, a liner for said body having an open ended reduced portion accessible through said opening, a closure cap for said opening having a portion enclosing the opening of the liner and a peripheral flange having a surface complementary to and fitting against the surface of the body around said opening and also closing the opening in said body.

MURRAY J. MACDONALD.

CARL SCHWENDLER.

CHRISTOPHER S. SCHWENDLER.

#### REFERENCES CITED

The following references are of record in the file of this patent:

#### UNITED STATES PATENTS

| Number    | Name                 | Date           |
|-----------|----------------------|----------------|
| 878,669   | Pianta               | Feb. 11, 1908  |
| 899,015   | Fitzsimmons          | Sept. 15, 1908 |
| 980,670   | Pepple               | Jan. 3, 1911   |
| 1,053,237 | Steel                | Feb. 18, 1913  |
| 1,417,534 | Leo                  | May 30, 1922   |
| 1,587,257 | Van Alstine          | June 1, 1926   |
| 1,861,552 | Savery               | June 7, 1932   |
| 1,891,361 | Stanley              | Dec. 20, 1932  |
| 1,940,771 | Prier                | Dec. 26, 1933  |
| 2,009,724 | Bircher              | July 30, 1935  |
| 2,218,047 | MacDonald et al.     | Oct. 15, 1940  |
| 2,235,617 | Klinzing             | Mar. 18, 1941  |
| 2,247,936 | Bishop               | July 1, 1941   |
| 2,285,614 | Rodgers, Jr., et al. | June 9, 1942   |